

J. Knight.

Making Hoes.

No 19,812.

Patented Mar 30, 1858.



Fig. 1.



Fig. 2.



Fig. 3.



Fig. 4.



Fig. 5.



Fig. 6.

Fig. 7.

Fig. 8.

Fig. 9.

Fig. 10.

# UNITED STATES PATENT OFFICE.

JUDSON KNIGHT, OF NEWARK, NEW JERSEY, ASSIGNOR TO S. BOYD, SAID  
BOYD ASSIGNOR TO R. W. BOOTH.

## IMPROVEMENT IN THE MANUFACTURE OF HOES.

Specification forming part of Letters Patent No. 19,812, dated March 30, 1858.

*To all whom it may concern:*

Be it known that I, JUDSON KNIGHT, of Newark, in the county of Essex and State of New Jersey, have invented a new and useful Improvement in the Manufacture of Hoes with Steel Blades and Malleable Cast-Iron Eyes; and I do hereby declare that the following is a full, clear, and exact description of the same, reference being had to the accompanying drawings, forming part of this specification.

This invention is an improvement on the hoe for which Letters Patent were granted to Samuel Boyd, January 13, 1857.

It consists in welding a plate of wrought-iron between the malleable cast-iron eye and the steel blade for the purpose of insuring a more perfect union of the eye and the blade.

Wrought-iron unites with steel and with malleable cast-iron more readily than steel and malleable cast-iron unite with each other, and hence the interposed wrought-iron plate serves as a medium for effecting a more perfect and secure union between the eye and the blade than can be effected when the malleable cast-iron and steel are in immediate contact.

To enable others to use my invention, I will proceed to describe the manner in which it is to be performed, with reference to the drawings, in which—

Figure 1 is a perspective view of a complete hoe constructed by my invention. Fig. 2 is a perspective view of the steel blade as it appears before the eye is applied to it. Fig. 3 is a perspective view of the malleable cast-iron eye as it appears before being united to the blade. Fig. 4 is a perspective view of the wrought-iron plate that is to be interposed between the steel blade and malleable cast-iron eye. Fig. 5 is a plan view representing the blade, the eye, and the wrought-iron plate as placed together ready for welding. Fig. 6 is a back view of the same. Fig. 7 is a central section of the same, taken transversely to the edge of the blade.

Similar letters of reference indicate corresponding parts in the several figures.

The blade A is cut to the required shape from a piece of cast-steel plate.

The eye B is cast with a flange, a, that is flat on the back side, which is to be attached to the front face of the blade.

The wrought-iron plate C, that is interposed between the eye and the blade, consists of a piece of sheet-iron of a thickness about one thirty-second of an inch, cut to a form to fit between the eye and its flange and the part of the blade to which they are to be united, with a margin, b, at its sides to be turned over on its front face.

The margin b represented in the drawings turns over far enough to lap over the edges of the flange of the eye, as shown in Fig. 5, where the said edges are indicated by dotted lines, and also in Figs. 6 and 7; but it is not necessary that the said margin should lap over the flange. All that is required is that its edges should fit up to the edges of the flange, so as to fill the corner or angular space formed between the latter edges and the face of the blade.

To unite the three pieces A, B, and C by welding, they are placed together, as shown in Figs. 5, 6, and 7, and heated to a proper welding-heat, and then placed, with the blade at the bottom, on an anvil under a drop containing a die of suitable form to fit the eye and its flange, and by the descent of the drop the three are united. The grinding up and bending of the blade are afterward performed in the usual manner.

I am aware that a wrought-iron plate has been applied in the form of a cap to assist in the union of the steel blade and malleable cast-iron eye of a hoe by the welding process, and therefore I do not claim the use of a wrought-iron uniting-plate when not interposed between the steel blade and malleable cast-iron eye; and I do not claim the lapping of the margin of the wrought-iron plate over the edges of the flange of the eye; but

What I claim as my invention, and desire to secure by Letters Patent, is—

The welding of the wrought-iron plate between the steel blade and the malleable cast-iron eye, substantially as and for the purpose set forth, or, in other words, I claim the hoe constructed of the three pieces A, B, and C, arranged relatively to each other and welded together substantially as herein specified.

JUDSON KNIGHT.

Witnesses:

SELIM FRAS. COHEN,  
JAMES F. BUCKLEY.